



US010288396B2

(12) **United States Patent**  
**Smith**

(10) **Patent No.:** **US 10,288,396 B2**  
(45) **Date of Patent:** **May 14, 2019**

(54) **NON-JACKETED BULLET AND METHOD OF MANUFACTURING A NON-JACKETED BULLET**

(71) Applicant: **Continuous Metal Technology, Inc.**, Ridgway, PA (US)

(72) Inventor: **Timothy G. Smith**, St. Marys, PA (US)

(73) Assignee: **Continuous Metal Technology, Inc.**, Ridgway, PA (US)

(\*) Notice: Subject to any disclaimer, the term of this patent is extended or adjusted under 35 U.S.C. 154(b) by 0 days.

(21) Appl. No.: **16/129,068**

(22) Filed: **Sep. 12, 2018**

(65) **Prior Publication Data**

US 2019/0003809 A1 Jan. 3, 2019

**Related U.S. Application Data**

(63) Continuation of application No. 15/664,282, filed on Jul. 31, 2017, now Pat. No. 10,107,605, which is a continuation-in-part of application No. 15/407,047, filed on Jan. 16, 2017, now Pat. No. 10,209,045.

(60) Provisional application No. 62/279,082, filed on Jan. 15, 2016.

(51) **Int. Cl.**

**F42B 12/00** (2006.01)

**F42B 12/74** (2006.01)

**F42B 12/34** (2006.01)

(52) **U.S. Cl.**

CPC ..... **F42B 12/74** (2013.01); **F42B 12/34**

(2013.01)

(58) **Field of Classification Search**

CPC ..... F42B 12/34; F42B 12/367  
See application file for complete search history.

(56) **References Cited**

U.S. PATENT DOCUMENTS

|                 |         |                     |
|-----------------|---------|---------------------|
| 2,409,307 A     | 10/1946 | Patch et al.        |
| 5,127,332 A     | 7/1992  | Corzine et al.      |
| 5,877,437 A     | 3/1999  | Oltrogge            |
| 5,945,629 A     | 8/1999  | Schildknecht et al. |
| 6,546,875 B2    | 4/2003  | Vaughn et al.       |
| 6,629,485 B2    | 10/2003 | Vaughn et al.       |
| 8,312,815 B1    | 11/2012 | Joys et al.         |
| 9,702,679 B2    | 7/2017  | Smith et al.        |
| 2004/0016356 A1 | 1/2004  | Jopson et al.       |
| 2004/0244629 A1 | 12/2004 | Jopson              |

FOREIGN PATENT DOCUMENTS

FR 2364427 A1 4/1978

Primary Examiner — Gabriel J. Klein

(74) Attorney, Agent, or Firm — The Webb Law Firm

(57) **ABSTRACT**

A non-jacketed bullet including a monolithic sintered body and a sintered projectile tip. The monolithic sintered body includes a base portion and a deformed hollow nose portion, and the sintered projectile tip includes a base portion and a nose portion. A portion of the sintered projectile tip extends into the deformed hollow nose portion of the monolithic sintered body and a portion of the sintered projectile tip extends from a distal end of the deformed hollow nose portion of the monolithic sintered body. Also, a method of manufacturing a non-jacketed bullet including providing a monolithic sintered body including a base portion and a hollow peripheral portion providing a sintered projectile tip, inserting a portion of the sintered projectile tip into the hollow portion of the monolithic sintered body, and forming the hollow peripheral portion into the shape of a hollow tapered nose.

**20 Claims, 15 Drawing Sheets**







FIG. 3



FIG. 4A



FIG. 4B



FIG. 5A



FIG. 5B



FIG. 6A



FIG. 6B



FIG. 7A



FIG. 7B



FIG. 8A

FIG. 8B



FIG. 9



FIG. 10



FIG. 11



FIG. 12



FIG. 13





FIG. 16



FIG. 17

**NON-JACKETED BULLET AND METHOD  
OF MANUFACTURING A NON-JACKETED  
BULLET**

**CROSS REFERENCE TO RELATED  
APPLICATION**

This application is continuation of U.S. patent application Ser. No. 15/664,282 filed on Jul. 31, 2017, which is a continuation-in-part of U.S. patent application Ser. No. 15/407,047 filed on Jan. 16, 2017, which claims priority to U.S. Provisional Application No. 62/279,082 filed on Jan. 15, 2016, the disclosures of which are hereby incorporated in their entirety by reference.

**BACKGROUND OF THE INVENTION**

**Field of the Invention**

The invention relates generally to non-jacketed bullets, and in particular, to non-jacketed bullets capable of being manufactured from lead-free materials, as well as methods of manufacturing such non-jacketed bullets.

**Description of Related Art**

The use of lead-based ammunition has been increasingly regulated in many states and countries. New, more restrictive lead bans have placed an emphasis on developing new lead-free projectiles and ammunition that represent cost-effective alternatives as compared to those that are presently available. In some cases, the implementation of regulations may be conditioned on the availability of cost-effective alternatives to lead-free projectiles.

Such lead projectiles and some lead-free projectiles are jacketed. In such jacketed projectiles, a casing of hard material surrounds the softer lead or lead-free solid projectile. Manufacturing of such jacketed projectiles involves many drawing and annealing steps to form a hollow cylinder made of the jacket material and then further processing is required to form the cylinder of jacket material around the lead or lead-free solid projectile. As such, the manufacturing process for these projectiles can be expensive and time consuming.

Therefore, there is a need for a non-jacketed projectile that can be made with a simpler manufacturing process at a reduced cost, and particularly, for a lead-free non-jacketed projectile that can be made in a cost effective manner.

**SUMMARY OF THE INVENTION**

The present invention is directed to an improved non-jacketed bullet and a method of manufacturing such a bullet. In one preferred and non-limiting embodiment or aspect, the improved non-jacketed bullet and the method of manufacturing the bullet address and/or overcome certain deficiencies and drawbacks associated with existing bullets and manufacturing processes by providing more efficient use of raw materials and/or reducing the number and/or difficulty of the processing steps in order to provide a cost-effective alternative to lead-based ammunition.

The present invention is directed to an improved non-jacketed bullet and a method of manufacturing such a bullet. In one non-limiting embodiment or aspect, the invention is directed to a non-jacketed bullet, comprising a monolithic sintered body and a sintered projectile tip. The base portion has a proximal end and a distal end and a deformed hollow nose portion extending distally from the distal end of the base portion, the sintered projectile tip has a base portion having a proximal end and a distal end and a nose portion

extending distally from the distal end of the base portion. A portion of the sintered projectile tip extends into the deformed hollow nose portion of the monolithic sintered body and a portion of the sintered projectile tip extends from a distal end of the deformed hollow nose portion of the monolithic sintered body.

In one non-limiting embodiment or aspect, at least one of the monolithic sintered body and the sintered projectile tip may comprise particles of a first metal and particles of a second metal and the particles of the first metal are bonded to the particles of the second metal by intermetallic compounds comprising the first metal and the second metal. In one non-limiting embodiment or aspect, at least one of the monolithic sintered body and the sintered projectile tip may comprise metallic particles that are connected by solid state bonds formed by compression and heat.

In one non-limiting embodiment or aspect, the porosity of the bullet may be 5-10%.

In one non-limiting embodiment or aspect, the monolithic sintered body and the projectile tip may be lead free. In one non-limiting embodiment or aspect, the monolithic sintered body may comprise at least one of copper, nickel, tin, zinc, or any combination thereof. In one non-limiting embodiment or aspect the monolithic sintered body may comprise copper or a copper-based alloy. In one non-limiting embodiment or aspect, the projectile tip may comprise iron. In one non-limiting embodiment or aspect, the projectile tip may comprise at least one of carbon, molybdenum, and copper.

In one non-limiting embodiment or aspect, the invention is directed to ammunition comprising a non-jacketed bullet according to one or more of the embodiments or aspects described above and a cartridge casing holding the non-jacketed bullet.

In one non-limiting embodiment or aspect, the present invention is directed to a method of manufacturing a non-jacketed bullet, the method comprising providing a monolithic sintered body comprising a base portion having a proximal end and a distal end and a hollow peripheral portion extending distally from the distal end of the base portion; providing a sintered projectile tip comprising a base portion having a proximal end and a distal end and a nose portion extending distally from the distal end of the base portion; inserting the base portion of the sintered projectile tip into the hollow portion of the monolithic sintered body; and forming the hollow peripheral portion into a shape of a hollow tapered nose while enclosing the base portion of the projectile tip within the hollow portion of the monolithic sintered body.

In one non-limiting embodiment or aspect, the provision of the monolithic sintered body may comprise providing a compacted powder preform a base portion having a proximal end and a distal end and a hollow peripheral portion extending distally from the distal end of the base portion and sintering the compacted powder preform. In one non-limiting embodiment or aspect, the provision of the sintered projectile tip may comprise providing a compacted powder preform a base portion having a proximal end and a distal end and a hollow peripheral portion extending distally from the distal end of the base portion and sintering the compacted powder preform. In one non-limiting embodiment or aspect, the provision of the compacted powder preform for the monolithic sintered body or the sintered projectile tip comprises providing powder to a cavity formed in a die between at least an upper punch and a lower punch and pressing the upper and lower punches together to compact the powder.

The non-jacketed bullet produced according to the method may have any of the aspects described above.

The present invention is neither limited to nor defined by the above summary. Rather, reference should be made to the claims for which protection is sought with consideration of equivalents thereto.

These and other features and characteristics of the present invention, as well as the methods of operation and functions of the related elements of structures and the combination of parts and economies of manufacture, will become more apparent upon consideration of the following description and the appended claims with reference to the accompanying drawings, all of which form a part of this specification, wherein like reference numerals designate corresponding parts in the various figures. It is to be expressly understood, however, that the drawings are for the purpose of illustration and description only and are not intended as a definition of the limits of the invention. As used in the specification and the claims, the singular form of "a", "an", and "the" include plural referents unless the context clearly dictates otherwise.

#### BRIEF DESCRIPTION OF THE DRAWINGS

FIG. 1 is a perspective view of a non-jacketed bullet according to a non-limiting embodiment or aspect of the present invention;

FIG. 2 is a sectional perspective view of the non-jacketed bullet of FIG. 1;

FIG. 3 is a sectional perspective view of a non-jacketed bullet according to a non-limiting embodiment or aspect of the present invention;

FIG. 4A is a perspective view of a monolithic sintered body with an internal cavity having a circular transverse cross-section before deformation according to a non-limiting embodiment or aspect of the present invention;

FIG. 4B is a sectional perspective view of the monolithic sintered body of FIG. 4A;

FIG. 5A is a perspective view of a monolithic sintered body with an internal cavity having a triangular transverse cross-section before deformation according to a non-limiting embodiment or aspect of the present invention;

FIG. 5B is a sectional perspective view of the monolithic sintered body of FIG. 5A;

FIG. 6A is a perspective view of a monolithic sintered body with an internal cavity having a square transverse cross-section before deformation according to a non-limiting embodiment or aspect of the present invention;

FIG. 6B is a sectional perspective view of the monolithic sintered body of FIG. 6A;

FIG. 7A is a perspective view of a monolithic sintered body with an internal cavity having a hexagonal transverse cross-section before deformation according to a non-limiting embodiment or aspect of the present invention;

FIG. 7B is a sectional perspective view of the monolithic sintered body of FIG. 7A;

FIG. 8A is a perspective view of a monolithic sintered body with an internal cavity having an octagonal transverse cross-section before deformation according to a non-limiting embodiment or aspect of the present invention;

FIG. 8B is a sectional perspective view of the monolithic sintered body of FIG. 8A;

FIG. 9 is a sectional view of a monolithic sintered body with an internal cavity having two portions before deformation according to a non-limiting embodiment or aspect of the present invention;

FIG. 10 is a sectional view of tooling for forming a compacted powder preform according to a non-limiting embodiment or aspect of the present invention;

FIG. 11 is a sectional perspective view of tooling for forming a compacted powder preform according to another non-limiting embodiment or aspect of the present invention;

FIG. 12 is a sectional perspective view of tooling for forming a compacted powder preform according to another non-limiting embodiment or aspect of the present invention;

FIG. 13 is a sectional view of a sizing/forming press according to a non-limiting embodiment or aspect of the present invention;

FIG. 14 is a perspective view of a non-jacketed bullet according to a non-limiting embodiment or aspect of the present invention;

FIG. 15 is a sectional perspective view of the non-jacketed bullet of FIG. 14;

FIG. 16 is a perspective view of a projectile tip according to a non-limiting embodiment or aspect of the present invention; and

FIG. 17 is a sectional view of a sizing/forming press according to a non-limiting embodiment or aspect of the present invention.

#### DETAILED DESCRIPTION OF THE INVENTION

Unless otherwise indicated, each numerical parameter in the specification and claims should be construed in light of the number of reported significant digits and by applying ordinary rounding techniques. Also, it should be understood that any numerical range recited herein is intended to include all sub-ranges subsumed therein. For example, a range of "1 to 10" is intended to include all sub-ranges between the recited minimum value of 1 and the recited maximum value of 10. All compositions are given in weight percent unless specifically stated otherwise.

It is to be understood that the invention may assume various alternative variations and step sequences, except where expressly specified to the contrary. It is also to be understood that the specific products, systems, and processes illustrated in the attached drawings, and described in the following specification, are simply exemplary embodiments of the invention. Hence, specific dimensions and other physical characteristics related to the embodiments disclosed herein are not to be considered as limiting. As used in the specification and the claims, the singular form of "a", "an", and "the" include plural referents unless the context clearly dictates otherwise.

The present invention is directed to a non-jacketed bullet. FIG. 1 illustrates a perspective view of a non-jacketed bullet according to a non-limiting embodiment or aspect of the present invention, and FIG. 2 illustrates a sectional perspective view of the non-jacketed bullet of FIG. 1.

As illustrated in FIGS. 1 and 2, and in one non-limiting embodiment or aspect, the non-jacketed bullet comprises a monolithic sintered body 10. The monolithic sintered body 10 may include a base portion 12 having a proximal end 14 and a distal end 16 and a hollow nose portion 18 extending distally from the distal end of the base portion 12.

In one non-limiting embodiment or aspect, the base portion 12 may include at least one transverse cross-section that is generally symmetric with respect to the central longitudinal axis of rotation L of the bullet. The cross-section may be circular. In another non-limiting embodiment or aspect, the entire base portion 12 may be generally

symmetric with respect to the central longitudinal axis of rotation L of the bullet to stabilize the trajectory of the bullet.

In one non-limiting embodiment or aspect, a distal portion 20 of the base portion 12 or the entire base portion 12 may be tapered axially inwardly in a distally extending direction. As a result, the transverse cross-sectional area of the base portion 12 decreases from the proximal end 14 of the base portion 12 to the distal end 16 of the base portion 12.

In one non-limiting embodiment or aspect, the base portion 12 may include at least one transverse cross section that is solid throughout. In another non-limiting embodiment or aspect, the entire base portion 12 may be solid throughout.

The hollow nose portion 18 comprises a proximal end 22, a distal end 24, and a sidewall 26 extending between the proximal end 22 and the distal end 24. The sidewall 26 defines at least one internal cavity 28. The hollow nose portion 18 may be formed into the shape of a hollow tapered nose such that the outer surface and/or the inner surface of the sidewall 26 of the hollow nose portion 18 taper axially inwardly from the proximal end 22 to the distal end 24. As a result, the transverse cross-sectional area of the internal cavity 28 decreases from the proximal end 22 of the hollow nose portion 18, adjacent to the base portion 12, to the distal end 24 of the hollow nose portion 18 and the transverse cross-sectional area defined by the outer perimeter of the hollow nose portion 18 decreases from the proximal end 22 of the hollow nose portion 18, adjacent to the base portion 12, to the distal end 24 of the hollow nose portion 18.

In one non-limiting embodiment or aspect, a portion of the hollow nose portion 18 or the entire hollow nose portion 18 may include at least one transverse cross-section that is generally symmetric with respect to the central longitudinal axis of rotation L of the bullet. In another non-limiting embodiment or aspect, the outer surface of the hollow nose portion 18 may be symmetric with respect to the central longitudinal axis of rotation L of the bullet to stabilize the trajectory of the bullet.

In one non-limiting embodiment or aspect, the internal cavity 28 of the hollow nose portion 18 may have a cylindrical transverse cross-section. In another non-limiting embodiment or aspect, the internal cavity 28 of the hollow nose portion 18 may have a transverse cross-section that is at least partly polygonal. In yet another non-limiting embodiment or aspect, the internal cavity 28 of the hollow nose portion 18 may have a transverse cross-section that is at least partly triangular, square, hexagonal, or octagonal. A triangular, square, or polygonal internal cavity 28 may facilitate the opening of the hollow nose portion 18 in sections to form distinct petals upon expansion when entering a target, such as tissue or simulated tissue. The internal cavity 28 of the hollow nose portion 18 may be configured and modified depending on the intended use. For example, an internal cavity 28 having a smaller cross-section and shorter length may result in deeper penetration and a smaller initial wound cavity. An internal cavity 28 having a larger cross-section and longer length may result in shorter penetration and a larger initial wound cavity. In one non-limiting embodiment or aspect, the internal cavity 28 may be generally symmetric with respect to the central longitudinal axis of rotation L of the bullet to stabilize the trajectory of the bullet.

In one non-limiting embodiment or aspect, as shown in FIG. 3, the monolithic sintered body 110 may have an internal cavity comprising a proximal portion 128a and a distal portion 128b. The proximal portion 128a of the internal cavity 128 may extend distally from the distal end 116 of the base portion 112 and the distal portion 128b of the

internal cavity 128 may extend distally from the proximal portion 128a. In one non-limiting embodiment or aspect, the proximal portion 128a of the internal cavity 128 may have a transverse cross-section that is circular forming a cylindrical internal cavity 128, while the inner surface of the distal portion 128b may taper inwardly in a distal direction such that the transverse cross-sectional area of the distal portion 128b of the internal cavity 128 decreases as it approaches the distal end 124 of the hollow nose portion 118. The maximum transverse cross-sectional area of the distal portion 128b of the internal cavity 128 may be larger than the maximum transverse cross-sectional area of the proximal portion 128a of the internal cavity 128. In one non-limiting embodiment or aspect, the distal portion 128b may first taper outwardly in a distal direction and then taper inwardly in a distal direction.

In non-limiting embodiments or aspects, the wall thickness of the sidewall of the hollow nose portion 18 may be less than half of a maximum radius of the base portion 12, for example, less than a third of the maximum radius of the base portion 12 or less than a quarter of the maximum radius of the base portion 12. Thinner wall thickness of the hollow tapered nose 18 may facilitate an opening of the hollow tapered nose 18 upon expansion when entering a target, such as tissue or simulated tissue.

In one non-limiting embodiment or aspect, the distal end 24 of the hollow nose portion 18 may be open into the internal cavity 28 of the hollow nose portion 18. In one non-limiting embodiment or aspect, the opening may have a transverse cross-section having the same shape as the cross-section of the internal cavity 28. The opening may facilitate expansion (mushrooming) of the hollow nose portion 18 on impact, increasing the diameter of the bullet to limit penetration and/or produce a larger diameter wound for faster incapacitation. In another non-limiting embodiment or aspect, the distal end 24 of the hollow nose portion 18 may be closed.

In one non-limiting embodiment or aspect, the base portion 12 and the hollow nose portion 18 of the monolithic sintered body 10 may be integrally formed together during a sintering process that applies heat and/or pressure to a compacted powder preform to form a unitary mass of material that includes solid-solid interfaces between adjacent powder particles. The monolithic nature of the monolithic sintered body 10 may provide better rotational stability compared to non-monolithic projectiles.

In one non-limiting embodiment or aspect, the hollow nose portion 18 may be tapered using a deformation process.

In one non-limiting embodiment or aspect, the material of the monolithic sintered body 10 may be any material capable of being sintered and deformed. In one non-limiting embodiment or aspect, the material of the monolithic sintered body 10 may be lead-free. In one non-limiting embodiment or aspect, the material of the monolithic sintered body 10 may include at least one of copper, nickel, tin, zinc, or combinations thereof. In one non-limiting embodiment or aspect, the monolithic sintered body may be made from copper or a copper-based alloy. In one non-limiting embodiment or aspect, the copper-based alloy may include at least 60% copper, for example, at least 70% copper, at least 80% copper, or at least 90% copper. In another non-limiting embodiment or aspect, the copper-based alloy may include at least one of nickel, tin, zinc, or any combination thereof to activate desired toughness and ductility. The ability to vary the mechanical properties via the composition gives flexibility and versatility. For example, varying the ductility can affect the depth of penetration of the bullet, the expansion

sion of the bullet, the fracture properties of the bullet and/or the penetration of the bullet into various surfaces. In one non-limiting embodiment or aspect, the material of the monolithic sintered body 10 may be a lead-free copper-based alloy that includes at least 70% copper and at least one of nickel, tin, zinc, or any combination thereof. In one non-limiting embodiment or aspect, the material of the monolithic sintered body 10 may be a lead-free copper-based alloy that includes at least 70% copper and the remainder zinc, for example, at least 80% copper and the remainder zinc, at least 90% copper and the remainder zinc, or at least 95% copper and the remainder zinc.

In one non-limiting embodiment or aspect, a method of manufacturing an bullet includes providing a monolithic sintered body including a base portion and a hollow peripheral portion extending distally from the base portion and forming the hollow peripheral portion into a hollow tapered nose.

FIG. 4A shows a perspective view of a monolithic sintered body 30 including a base portion 32 and a hollow peripheral portion 34 extending distally from the base portion 32 prior to forming the hollow peripheral portion 34 into a hollow tapered nose according to one non-limiting embodiment or aspect. FIG. 4B shows a sectional perspective view of the monolithic sintered body 30 of FIG. 4A. The hollow peripheral portion 34 has an internal cavity 33 having a circular cross-section.

FIG. 5A shows a perspective view of a monolithic sintered body 130 including a base portion 132 and a hollow peripheral portion 134 extending distally from the base portion 132 prior to forming the hollow peripheral portion 134 into a hollow tapered nose according to one non-limiting embodiment or aspect. FIG. 5B shows a sectional perspective view of the monolithic sintered body 130 of FIG. 5A. The hollow peripheral portion 134 has an internal cavity 133 having a triangular cross-section.

FIG. 6A shows a perspective view of a monolithic sintered body 230 including a base portion 232 and a hollow peripheral portion 234 extending distally from the base portion 232 prior to forming the hollow peripheral portion 234 into a hollow tapered nose according to one non-limiting embodiment or aspect. FIG. 6B shows a sectional perspective view of the monolithic sintered body 230 of FIG. 6A. The hollow peripheral portion 234 has an internal cavity 233 having a square cross-section.

FIG. 7A shows a perspective view of a monolithic sintered body 330 including a base portion 332 and a hollow peripheral portion 334 extending distally from the base portion 332 prior to forming the hollow peripheral portion 334 into a hollow tapered nose according to one non-limiting embodiment or aspect. FIG. 7B shows a sectional perspective view of the monolithic sintered body 330 of FIG. 7A. The hollow peripheral portion 334 has an internal cavity 333 having a hexagonal cross-section.

FIG. 8A shows a perspective view of a monolithic sintered body 430 including a base portion 432 and a hollow peripheral portion 434 extending distally from the base portion 432 prior to forming the hollow peripheral portion 434 into a hollow tapered nose according to one non-limiting embodiment or aspect. FIG. 8B shows a sectional perspective view of the monolithic sintered body 430 of FIG. 8A. The hollow peripheral portion 434 has an internal cavity 433 having an octagonal cross-section.

In one non-limiting embodiment or aspect, a proximal portion of the internal cavity of the hollow peripheral portion may extend distally from the distal end of the base portion and a distal portion of the internal cavity may extend

distally from the proximal portion. The proximal portion may have a different transverse cross-sectional area and/or shape from the distal portion. Each of the proximal portion and the distal portion may have a transverse cross-section that is triangular, square, hexagonal, or octagonal. The maximum transverse cross-sectional area of the distal portion of the internal cavity may be larger than the maximum transverse cross-sectional area of the proximal portion of the internal cavity. The distal portion may have two sections where the first section tapers outwardly in a distally extending direction from the proximal portion 533a and the second section has no taper.

In one non-limiting embodiment or aspect, the proximal portion may have a transverse cross-section that is circular.

FIG. 9 shows a sectional view of a monolithic sintered body 530 including a base portion 532 and a hollow peripheral portion 534 extending distally from the base portion 532 prior to forming the hollow peripheral portion 534 into a hollow tapered nose according to one non-limiting embodiment or aspect. The proximal portion 533a of the internal cavity 533 has a transverse cross-section that is circular, while the transverse cross-section of the distal portion 533b of the internal cavity 533 is hexagonal. The maximum transverse cross-sectional area of the distal portion 533b of the internal cavity 533 is larger than the maximum transverse cross-sectional area of the proximal portion 533a of the internal cavity 533. The distal portion 533b has two sections where the first section tapers outwardly in a distally extending direction from the proximal portion 533a and the second section has no taper.

In one non-limiting embodiment or aspect, a portion of the distal end of the base portion 32 may have a constant outside diameter or may taper axially inwardly in a distally extending direction.

In one non-limiting embodiment or aspect, the hollow peripheral portion 34 may have an outer surface with a constant outside diameter or an outer surface that tapers axially inwardly in a distally extending direction.

In one non-limiting embodiment or aspect, the hollow peripheral portion 34 may have an inner surface with a constant inside diameter or an inner surface that tapers axially inwardly in a distally extending direction.

In one non-limiting embodiment or aspect, the hollow peripheral portion 34 may be formed into the shape of a hollow tapered nose by a deformation process. In one preferred and non-limiting embodiment or aspect, the entire hollow peripheral portion 34 may be formed into the shape of a hollow tapered nose by a deformation process. In one non-limiting embodiment or aspect, the hollow peripheral portion 34 and a portion of the base portion 32 may be formed into a hollow tapered nose, as shown in FIGS. 1 and 2, by a deformation process.

In one non-limiting embodiment or aspect, the method of manufacturing an bullet may include providing powder to a cavity formed in a die between at least an upper punch and a lower punch to form a compacted powder preform including a base portion and a hollow peripheral portion extending distally from the base portion. In one non-limiting embodiment or aspect, the powder may be any material capable of being sintered and deformed. In one non-limiting embodiment or aspect, the powder may be selected from gas atomized powder or water atomized powder. In one non-limiting embodiment or aspect, the powder may be lead free. In one non-limiting embodiment or aspect, the powder may comprise at least one of copper, nickel, tin, zinc, or combinations thereof. In one non-limiting embodiment or aspect, the powder may comprise copper or a copper-based alloy. In

one non-limiting embodiment or aspect, the copper-based alloy powder may include at least 60% copper, for example, at least 70% copper, at least 80% copper, or at least 90% copper. In another non-limiting embodiment or aspect, the copper-based alloy powder may include at least one of nickel, tin, zinc, or any combination thereof to activate desired toughness and ductility. In one non-limiting embodiment or aspect, the powder may comprise a lead-free copper-based alloy that includes at least 70% copper and at least one of nickel, tin, zinc, or any combination thereof. In one non-limiting embodiment or aspect, the lead-free copper-based alloy that includes at least 70% copper and the remainder zinc, for example, at least 80% copper and the remainder zinc, at least 90% copper and the remainder zinc, or at least 95% copper and the remainder zinc. As an example, the powder may be water atomized Accu-powder 165A, which comprises 95% copper and a remainder of zinc with a particle size of 20-100  $\mu\text{m}$ . The ability to vary the mechanical properties via the composition gives flexibility and versatility. For example, varying the ductility can affect the depth of penetration of the bullet, the expansion of the bullet, the fracture properties of the bullet, and/or the penetration of the bullet into various surfaces.

Particle size of the constituent powder can be at least 5  $\mu\text{m}$  and up to 500  $\mu\text{m}$ , for example, 5-500  $\mu\text{m}$ , 20-300  $\mu\text{m}$ , or 20-100  $\mu\text{m}$ .

In one non-limiting embodiment or aspect, the powder may be mixed with a lubricant to allow the powder particles to move relative to other particles and relative to tooling. For example, atomized wax may be used, such as Acrawax A. At least 0.2 wt. % and up to 2.0 wt. % of the lubricant may be provided, for example, 0.2-2.0 wt. %, 0.2-1.0 wt. %, or 0.5 wt. %. The lubricant may be blended together in a conical blender for 20 minutes to allow for homogenization.

In one non-limiting embodiment or aspect, FIGS. 10 and 11 show sectional views of tooling for forming a compacted powder preform. The tooling may include a die 36, an upper punch 38, and a lower punch 40, 140 having two sections. The die 36 may include an internal through-hole 42 which may be cylindrical. The transverse cross-sectional area of the through-hole 42 may be uniform. A lower end of the upper punch 38 may have a size and shape corresponding to a size and shape of an upper portion of the through-hole 42 of the die 36 such that the lower end of the upper punch 38 can fit into the through-hole 42 of the die 36 while not allowing powder to pass between the die 36 and the upper punch 38. The size and shape of the through-hole of the die 36 and the size and shape of the lower end of the upper punch 38 may correspond to the desired size and shape of the base portion of the compacted powder preform.

The first section 44 of the lower punch 40 may have a size and shape corresponding to a size and shape of the lower portion of the through-hole 42 of the die 36 such that the first section 44 of the lower punch 40 can fit into the through-hole 42 of the die 36 while not allowing powder to pass between the die 36 and the first portion 44 of the lower punch 40. The second section 46 of the lower punch 40 has a size and shape corresponding to the size and shape of the internal cavity that is desired in the hollow peripheral portion of the compacted powder preform. For example, the second section 46 of the lower punch 40 has a transverse cross-section that is triangular, square, hexagonal, or octagonal.

In one non-limiting embodiment or aspect, the second section 46 of the lower punch 40 may comprise two portions each having a different transverse cross-sectional area and/or shape in order to form a bullet having an internal cavity with two portions as described above. Each of the first portion

and the second portion may have a transverse cross-section that is triangular, square, hexagonal, or octagonal. The maximum transverse cross-sectional area of the distal portion of the internal cavity may be larger than the maximum transverse cross-sectional area of the proximal portion of the internal cavity. The second portion may have two sections where the first section tapers outwardly in a distally extending direction from the first portion and the second section has no taper.

10 In one non-limiting embodiment or aspect, FIG. 12 shows tooling where the second section 146 of the lower punch 140 has portions. The first portion 146a has a circular transverse cross-section and the second portion 146b has a hexagonal transverse cross-section. The second portion 146b includes a section that tapers outwardly in a distally extending direction from the first portion 146a.

The first section 44 of the lower punch 40 and the second section 46 of the lower punch 40 may be separate from one another or may be integral.

20 In one non-limiting embodiment or aspect shown in FIG. 10, the second section 46 of the lower punch 40 passes through an internal passageway 48 in the first section 44 of the lower punch 40 and extends distally beyond the distal end of the first section 44 of the lower punch 40. The second section 46 of the lower punch 40 has a circular transverse cross-section forming a cylindrical internal cavity in the hollow peripheral portion of the compacted powder preform.

25 In another non-limiting embodiment or aspect shown in FIG. 11, the second section 46 of the lower punch 40 is integral with the first section 44 of the lower punch 40 and has a hexagonal transverse cross-section forming an internal cavity having a hexagonal transverse cross-section in the hollow peripheral portion of the compacted powder preform as shown in FIGS. 7A and 7B.

30 In either embodiment or aspect, the sidewall of the hollow peripheral portion of the compacted powder preform is formed between the top surface of the first section 44 of the lower punch 40, the outer surface of the second section 46 of the lower punch 40, and the inner surface of the through-hole 42 of the die 36. The base portion of the compacted powder preform is formed between the bottom surface of the upper punch 38, the top surface of the second portion 46 of the lower punch 40, and the inner surface of the through-hole 42 of the die 36. In one non-limiting embodiment or aspect, the first section 44 and the second section 46 of the lower punch 40 may be separate pieces as shown in FIG. 10. In another non-limiting embodiment or aspect, the first section 44 and the second section 46 of the lower punch 40 may be integral as shown in FIG. 11. In yet another non-limiting embodiment or aspect, the second section 46 of the lower punch 40 may be in a sliding relationship with the first section 44 of the lower punch 40.

35 In one non-limiting embodiment or aspect, the die 36 and the upper punch 38 may be made of tool steel. In another non-limiting embodiment or aspect, the die 36, the upper punch 38, and the lower punch 40 may be made of tool steel.

40 In one preferred and non-limiting embodiment or aspect, the through-hole 42 in the die 36 may be a cylindrical cavity.

To form the compacted powder preform, powder may be provided to the cavity formed by the die 36, the bottom end of the upper punch 38, and the top end of the lower punch 40, and at least the upper punch 38 may be pressed to compact the powder. In one preferred and non-limiting embodiment or aspect, the powder may be compacted to form the compacted powder preform by moving the upper punch 38 and/or the lower punch 40 into the through-hole 42 of the die 36 such that the powder is compacted between the

## 11

upper punch 38 and the lower punch 40. In one non-limiting embodiment or aspect, the upper punch 38 may enter the die 36 and exert 20-60 tons per square inch of pressure onto the powder. In one preferred and non-limiting embodiment or aspect, the tooling may be placed in a uniaxial compaction press such as a 30 ton Gasbarre mechanical press.

After compaction, the compacted powder preform (green preform) may be ejected via the lower punch 40 and placed in a sintering furnace.

In one preferred and non-limiting embodiment or aspect, the compacted powder preform may be heated to a temperature below the melting point of its main constituent for a time sufficient to form and grow necks between adjacent powder particles such that sufficient ductility is provided for a subsequent step where the hollow peripheral portion and, optionally, a portion of the base portion is deformed into the shape of a hollow tapered nose.

In one non-limiting embodiment or aspect, the time and temperature of sintering may be adjusted to adjust the desired mechanical properties of the bullet. In one non-limiting embodiment or aspect, the sintering temperature may be at least 1500° F. and at most 2000° F., for example, 1500-2000° F., 1600-2000° F., or 1600-1950° F. However, other conditions, such as composition of the compacted powder preform, may require sintering temperatures outside of 1500° F. and 2000° F. In one non-limiting embodiment or aspect, the compact may be heated to a final sintering temperature of about 1900° F. and held for about 60 minutes.

By way of non-limiting examples, Table 1 shows the sintering temperatures for four brass powders comprising copper and zinc and a copper powder.

TABLE 1

| Copper (wt. %) | Zinc (wt. %) | Sintering Temperature (° F.) |
|----------------|--------------|------------------------------|
| 70             | 30           | 1620                         |
| 80             | 20           | 1670                         |
| 90             | 10           | 1800                         |
| 95             | 5            | 1900                         |
| 100            | 0            | 1950                         |

In one non-limiting embodiment or aspect, the compacted powder preform may be sintered in a non-oxidizing or reducing atmosphere, for example, a vacuum atmosphere or a gas atmosphere comprising nitrogen, hydrogen, inert gases, or mixtures thereof.

In one non-limiting example, the compacted powder preform is sintered in a belt feed sintering furnace with a controlled temperature profile and reducing atmosphere. For example, an Abbott furnace company 4 zone 20" sintering furnace may be used. The atmosphere may be a nitrogen-hydrogen mix with varied gas flows of nitrogen and hydrogen at various points in the furnace.

In one preferred and non-limiting embodiment or aspect, the method of manufacturing an bullet may include deforming the hollow peripheral portion 34 of the monolithic sintered body 30 into the shape of a hollow tapered nose and/or reduce the porosity of the hollow peripheral portion 34, such as by a mechanical deformation in a sizing/forming press.

In one non-limiting embodiment or aspect, a deformation process may be further applied to the base portion 32 to shape the base portion 32 and/or to reduce porosity of the base portion 32.

According to one non-limiting embodiment or aspect, FIG. 13 shows a sectional view of a sizing/forming press for forming the hollow peripheral portion 34, and, optionally,

## 12

portion of the base portion 32 into the shape of a hollow tapered nose. The sizing/forming press may include a die 50 and a punch 52. The die 50 has an internal cavity 54 having a shape corresponding to the desired shape of the final monolithic sintered body. In one non-limiting embodiment or aspect, the die 50 may have a cylindrical cavity with a tapered, generally conical end to give the monolithic sintered body 30 its final shape, including a hollow tapered nose portion, while retaining the internal cavity of the monolithic sintered body 30.

The monolithic sintered body 30 is placed into the internal cavity 54 of the die 50 and the punch 52 is inserted into the internal cavity 54 of the die, thereby forcing the monolithic sintered body 30 to deform and contour to the shape of the internal cavity 54 of the die 50. The transverse cross-sectional area of the outer surface of the hollow nose portion 18 is only minimally changed at the proximal end 22, but is reduced significantly at the distal end 24, thereby closing or nearly closing the distal end 24 of the hollow nose portion 18. The shape of the internal cavity 28 of the hollow nose portion 18 after deformation is determined by the shape of the hollow peripheral portion 34 of the monolithic sintered body 30 prior to forming. When the transverse cross-section of the hollow peripheral portion 34 of the monolithic sintered body 30 prior to forming is triangular, square, hexagonal, or octagonal, the inner surface of the hollow peripheral portion 34 folds inwardly during the deformation such that the inner surface of the internal cavity 28 of the monolithic sintered body 30 after deformation may have portions that taper outwardly in a distal direction and portions that taper inwardly in a distal direction. The combination of the shape of the internal cavity 33 of the hollow peripheral portion 34 and the deformation of the hollow peripheral portion 34 provides a non-jacketed bullet having a cavity with a unique shape that is larger than prior art non-jacketed bullets.

In one non-limiting embodiment or aspect, the deformation of the hollow peripheral portion 34 into the shape of a hollow tapered nose restricts the outside dimension and also forms the conical nose (ogive) of the bullet while maintaining the internal hollow cavity for increased expansion.

In one preferred and non-limiting embodiment or aspect, FIG. 13 further illustrates a holder 56 for holding the monolithic sintered body 30 during insertion of the monolithic sintered body 30 and the punch 52 into the die 50. In another non-limiting embodiment or aspect, FIG. 13 further illustrates a pin 58 for facilitating the release of the monolithic sintered body 30 from the die 50 after forming the hollow peripheral portion 34 into the shape of a hollow tapered nose.

After the monolithic sintered body 30 is released from the die 50, the monolithic sintered body 30 may be deburred, such as by vibratory or rotary deburring, to remove burrs, polish the edges, and ready the bullet for loading into ammunition.

FIG. 14 illustrates a perspective view of a non-jacketed bullet according to another non-limiting embodiment or aspect of the present invention, and FIG. 15 illustrates a sectional perspective view of the non-jacketed bullet of FIG. 14.

As illustrated in FIGS. 14 and 15, the non-jacketed bullet comprises any of the monolithic sintered bodies 210 described above and a projectile tip 60. The projectile tip 60, shown in FIG. 16, may include a base portion 62 having a proximal end 64 and a distal end 66 and a nose portion 68 extending distally from the distal end 66 of the base portion 62.

## 13

In one non-limiting embodiment or aspect, the base portion **62** may be generally symmetric with respect to the central longitudinal axis of rotation **L** of the bullet to stabilize the trajectory of the bullet. The cross-section of the base portion **62** may be circular, and the base portion **62** may have a substantially cylindrical shape.

In one non-limiting embodiment or aspect, the base portion **62** may include at least one transverse cross section that is solid throughout. In another non-limiting embodiment or aspect, the entire base portion **62** may be solid throughout.

The nose portion **68** comprises a proximal end **70** and a distal end **72**. The nose portion **68** has a substantially conical shape such that the outer surface of the nose portion **68** tapers axially inwardly from the proximal end **70** to the distal end **72**. As a result, the transverse cross-sectional area of the nose portion **68** decreases from the proximal end **70** of the nose portion **68**, adjacent to the base portion **62**, to the distal end **72** of the nose portion **68**.

In one non-limiting embodiment or aspect, the base portion **62** of the projectile tip **60** may be integrally formed together during a sintering process that applies heat and/or pressure to a compacted powder preform to form a unitary mass of material.

In one non-limiting embodiment or aspect, the material of the projectile top **60** may be any material capable of being sintered and deformed. In one non-limiting embodiment or aspect, the material of the projectile tip **60** may be lead-free. In one non-limiting embodiment or aspect, the material of the projectile tip **60** may include iron and at least one of carbon, molybdenum, and copper. In one non-limiting embodiment or aspect, the iron-based alloy may include at least 60% iron, for example, at least 90% iron or at least 95% iron. In another non-limiting embodiment or aspect, the iron-based alloy may include up to 5% carbon, for example, up to 0.75% carbon. While no carbon need be added to the iron-based alloy, in one non-limiting embodiment or aspect, at least 0.5% carbon may be added, for example, at least 0.3% carbon. The iron based alloy may include 0-5% carbon or 0.3-0.75% carbon. While no additional alloying elements need be added to the iron-based alloy, in one non-limiting embodiment or aspect, at least 0.8% molybdenum and up to 0.9% molybdenum, for example, 0.8-0.9% molybdenum or 0.85% molybdenum may be included in the iron-based alloy and/or at least 1.5% copper and up to 2.5% copper, for example, 1.5-2.5% copper, 1.75-2.25% copper, or 2% copper may be included in the iron-based alloy. In one non-limiting embodiment or aspect, the material of the projectile tip **60** may be an iron-based alloy that includes 95% iron and the remainder carbon, for example, at least 97.5% iron and the remainder carbon, or at least 99% iron and the remainder carbon.

In one non-limiting embodiment or aspect, the method of manufacturing a bullet may include providing powder to a cavity formed in a die between at least an upper punch and a lower punch to form a compacted powder preform. In one non-limiting embodiment or aspect, the powder may be any material capable of being sintered and deformed. In one non-limiting embodiment or aspect, the powder may be selected from gas atomized powder or water atomized powder. In one non-limiting embodiment or aspect, the powder may be lead-free. In one non-limiting embodiment or aspect, the powder may be an iron-based alloy powder comprising iron and at least one of carbon, molybdenum, and copper. In one non-limiting embodiment or aspect, the iron-based alloy powder may include at least 60% iron, for example, at least 95% iron, at least 97.5% iron, or at least 99% iron. In another non-limiting embodiment or aspect, the

## 14

iron-based alloy powder may include at least one of molybdenum or copper. In one non-limiting embodiment or aspect, the lead-free iron-based alloy powder may include at least 95% iron and the remainder carbon, for example, at least 97.5% iron and the remainder carbon or at least 99% iron and the remainder carbon. In another non-limiting embodiment or aspect, an iron or iron-alloy powder may be mixed with a carbon powder, such as graphite.

10 Particle size of the constituent iron or iron-based alloy powder can be at least 10  $\mu\text{m}$  and up to 300  $\mu\text{m}$ , for example, 10-300  $\mu\text{m}$ , 10-100  $\mu\text{m}$ , or 20-100  $\mu\text{m}$ . Particle size of the constituent carbon powder can be at least 0.5  $\mu\text{m}$  and up to 100  $\mu\text{m}$ , for example, 0.5-100  $\mu\text{m}$ , 1-5  $\mu\text{m}$ , or 1  $\mu\text{m}$ .

15 In one non-limiting embodiment or aspect, the powder may be mixed with a lubricant to allow the powder particles to move relative to other particles and relative to tooling. For example, atomized wax may be used, such as Acrawax A. At least 0.25% and up to 5.0% of the lubricant may be provided, for example, 0.25-5.0%, 0.3-0.75%, or 0.5%. The lubricant and the powder may be blended together in a conical blender for 20 minutes to allow for homogenization.

20 In one non-limiting embodiment or aspect, a compacted powder preform having the final desired shape is formed from the powder in a similar manner to the compacted powder preform for the body of the bullet that is described above.

25 In one preferred and non-limiting embodiment or aspect, the compacted powder preform may be heated to a temperature below the melting point of its main constituent for a time sufficient to form and grow bonds between adjacent powder particles.

30 In one non-limiting embodiment or aspect, the time and temperature of sintering may be adjusted to adjust the desired mechanical properties of the bullet. In one non-limiting embodiment or aspect, the sintering temperature may be at least 1400° F. and at most 2600° F., for example, 1400-2600° F., 1900-2300° F., or 2050° F. However, other conditions, such as composition of the compacted powder preform, may require sintering temperatures outside of 1400° F. and 2600° F.

35 In one non-limiting embodiment or aspect, the sintering time may be at least 10 minutes and up to 60 minutes, for example, 10-60 minutes, 20-60 minutes, or 45 minutes.

40 In one non-limiting embodiment or aspect, the compacted powder preform may be sintered in a non-oxidizing or reducing atmosphere, for example, a vacuum atmosphere or a gas atmosphere comprising nitrogen, hydrogen, inert gases, or mixtures thereof. The sintering atmosphere may be 100 vol. % hydrogen or may be a hydrogen/nitrogen mixture with at least 25 vol. % hydrogen, for example, 25-50 vol. % hydrogen and 50-75 vol. % nitrogen or 25 vol. % hydrogen and 75 vol. % nitrogen.

45 In one non-limiting example, the compacted powder preform is sintered in a belt feed sintering furnace with a controlled temperature profile and reducing atmosphere. For example, an Abbott furnace company 4 zone 20" sintering furnace may be used.

50 In one preferred and non-limiting embodiment or aspect, the method of manufacturing a bullet may include inserting the sintered projectile tip **60** into the internal cavity **33** of the undeformed monolithic sintered body **30** and deforming the hollow peripheral portion **34** of the monolithic sintered body **30** into the shape of a hollow tapered nose and/or reducing the porosity of the hollow peripheral portion **34**, such as by a mechanical deformation in a sizing/forming press.

## 15

In one non-limiting embodiment or aspect, a deformation process may be further applied to the base portion 32 to shape the base portion 32 and/or to reduce porosity of the base portion 32.

According to one non-limiting embodiment or aspect, FIG. 17 shows a sectional view of a sizing/forming press for forming the hollow peripheral portion 34, and, optionally, a portion of the base portion 32 of the monolithic sintered body 30 into the shape of a hollow tapered nose. In FIG. 17, the bullet is being removed from the sizing/forming press after deformation. The sizing/forming press may include a die 150, a pin 158, and a punch 152. The die 150 has an internal cavity 154 having a shape corresponding to the desired shape of the final bullet. In one non-limiting embodiment or aspect, the die 150 may have a cylindrical cavity with a tapered, generally conical end to give the monolithic sintered body 30 its final shape, including a hollow tapered nose portion, while sealing the projectile tip 60 within the internal cavity 33 of the monolithic sintered body 30.

The monolithic sintered body 30 is deformed in the sizing/forming press in the same manner as was described above with respect to the bullet that does not include a projectile tip.

With respect to the sintering of both the monolithic sintered body and the penetrator tip, in one non-limiting embodiment or aspect, the sintering step is a liquid phase sintering process. The liquid phase sintering process can be performed at a temperature at least above the solidus of one of the materials. In one contemplated liquid phase sintering process, the performed monolithic body or the preformed penetrator top comprise at least two metallic components (e.g., formed from a mixture of blended metallic powders as described above), bonding occurs as the temperature is elevated above the eutectic temperature of two materials and a temporary liquid is formed. As soon as the liquid forms, it alloys with the other metal and the melting point rises such that there is no longer liquid. The result is light metal-to-metal bonding that relies on the small, weak, and brittle intermetallic compounds that form at the contact points of the particles as a result of passing through the eutectic temperature.

In one non-limiting embodiment or aspect, a solid state sintering process may be used. For example, a solid state sintering process can be used for a bullet made of pre-alloyed materials or elemental materials. In one embodiment of the solid state sintering process, the sintering process occurs at a temperature below the solidus of the constituent materials. Specifically, particles form bonds along the regions that have been forced into close contact during pressing or compacting of these particles. Bonding occurs by atoms moving into the vacancies between particle boundaries. However, the particles are essentially the same size and shape before and after the sintering process. Dimensional changes of the compacted mixture are small. In addition, no liquid metal is present at any stage during the solid state sintering process. During the solid state sintering process, neutral or slightly reducing atmospheres can be used, since the oxide layer on the outside of the powdered particles is mechanically smeared during the pressing operation which prepares the metal in these regions for sinter bonding.

In one non-limiting embodiment or aspect, the bullet, either with or without a penetrator tip, may have a porosity of between about 2 to about 20%. For example, in the green state, the compacted powder preform may have a porosity of about 20%. In the sintered state, the monolithic sintered body may have a porosity of about 10-15%. After deforma-

## 16

tion, the bullet may have a porosity of about 5-10%. It is believed that, as the monolithic sintered body is deformed, large pores may collapse and the density of the part may increase. The porosity allows the bullet to deform as it contacts the engraved grooves in the barrel of the firearm. Conversely, when jacketed bullets are used, material is removed by engraved grooves in the barrel of the firearm.

In one non-limiting embodiment or aspect, ammunition is provided, which may include a non-jacketed bullet according to one or more embodiments or aspects described above and a cartridge casing holding the non-jacketed bullet. In another non-limiting embodiment or aspect, the ammunition may further include a priming compound and/or gunpowder.

Although the invention has been described in detail for the purpose of illustration based on what is currently considered to be the most practical and preferred embodiments, it is to be understood that such detail is solely for that purpose and that the invention is not limited to the disclosed embodiments, but, on the contrary, is intended to cover modifications and equivalent arrangements that are within the spirit and scope of the description. For example, it is to be understood that the present invention contemplates that, to the extent possible, one or more features of any embodiment can be combined with one or more features of any other embodiment.

The invention claimed is:

1. A bullet, comprising:

a monolithic sintered body comprising:

a base portion having a proximal end and a distal end; and

a deformed hollow nose portion extending distally from the distal end of the base portion; and

a sintered projectile tip comprising:

a base portion having a proximal end and a distal end; and

a nose portion extending distally from the distal end of the base portion,

wherein a portion of the sintered projectile tip extends into the deformed hollow nose portion of the monolithic sintered body and a portion of the sintered projectile tip extends from a distal end of the deformed hollow nose portion of the monolithic sintered body and

wherein the bullet is non-jacketed and expandable, and the deformed hollow nose portion is ductile such that, upon impact, the deformed hollow nose portion expands to form distinct petals.

2. The bullet of claim 1, wherein at least one of the monolithic sintered body and the sintered projectile tip comprise particles of a first metal and particles of a second metal and the particles of the first metal are bonded to the particles of the second metal by intermetallic compounds comprising the first metal and the second metal.

3. The bullet of claim 1, wherein at least one of the monolithic sintered body and the sintered projectile tip comprise metallic particles that are connected by solid state bonds formed by compression and heat.

4. The bullet of claim 1, wherein the porosity of the bullet is 5-10%.

5. The bullet of claim 1, wherein the monolithic sintered body and the projectile tip are lead free.

6. The bullet of claim 1, wherein the monolithic sintered body comprises at least one of copper, nickel, tin, zinc, or any combination thereof.

7. The bullet of claim 1, wherein the monolithic sintered body comprises copper or a copper-based alloy.

## 17

8. The bullet of claim 1, wherein the projectile tip comprises iron.
9. The bullet of claim 8, wherein the projectile tip comprises at least one of carbon, molybdenum, and copper.
10. Ammunition, comprising:  
a bullet according to claim 1; and  
a cartridge casing holding the bullet.
11. A method of manufacturing a bullet according to claim 1, the method comprising:  
providing a monolithic sintered body comprising:  
a base portion having a proximal end and a distal end;  
and  
a hollow peripheral portion extending distally from the distal end of the base portion;  
providing a sintered projectile tip comprising:  
a base portion having a proximal end and a distal end;  
and  
a nose portion extending distally from the distal end of the base portion;  
inserting the base portion of the sintered projectile tip into the hollow portion of the monolithic sintered body;  
forming the hollow peripheral portion into a shape of a hollow tapered nose while enclosing the base portion of the projectile tip within the hollow portion of the monolithic sintered body;  
wherein a portion of the sintered projectile tip extends into the deformed hollow nose portion of the monolithic sintered body and a portion of the sintered projectile tip extends from a distal end of the deformed hollow nose portion of the monolithic sintered body and wherein the bullet is non-jacketed and expendable, and the deformed hollow nose portion is ductile such that, upon impact, the deformed hollow nose portion extends to form distinct petals.
12. The method of claim 11, wherein providing the monolithic sintered body comprises:  
providing a compacted powder preform comprising:

## 18

- a base portion having a proximal end and a distal end;  
and  
a hollow peripheral portion extending distally from the distal end of the base portion; and  
sintering the compacted powder preform.
13. The method of claim 11, wherein providing the projectile tip comprises:  
providing a compacted powder preform comprising:  
a base portion having a proximal end and a distal end;  
and  
a nose portion extending distally from the distal end of the base portion; and  
sintering the compacted powder preform.
14. The method of claim 12, wherein providing the compacted powder preform includes:  
providing a powder to a cavity formed in a die between at least an upper punch and a lower punch; and  
pressing the upper and lower punches together to compact the powder.
15. The method of claim 13, wherein providing the compacted powder preform includes:  
providing a powder to a cavity formed in a die between at least an upper punch and a lower punch; and  
pressing the upper and lower punches together to compact the powder.
16. The method of claim 11, wherein the monolithic sintered body and the projectile tip are lead free.
17. The method of claim 11, wherein the monolithic sintered body comprises at least one of copper, nickel, tin, zinc, or any combination thereof.
18. The method of claim 11, wherein the monolithic sintered body comprises copper or a copper-based alloy.
19. The method of claim 11, wherein the projectile tip comprises iron.
20. The method of claim 11, wherein the projectile tip comprises at least one of carbon, molybdenum, and copper.

\* \* \* \* \*